

## UNITED STATES PATENT OFFICE

2,396,569

## METHOD OF PURIFYING ELECTROLYTES

Dinsmore Laurence Griffith and Luther Glenn Hendrickson, Flin Flon, Manitoba, Canada, assignors to Hudson Bay Mining and Smelting Company Limited, Winnipeg, Manitoba, Canada, a corporation of Canada

No Drawing. Application August 9, 1943, Serial No. 497,980

2 Claims. (Cl. 23—50)

The present invention relates to a method of purifying electrolytes. More particularly, it relates to a method of purifying zinc electrolytes and especially to electrolytes as used in the electrolytic method of winning zinc from ores or other materials.

That certain impurities in electrolytes cause great difficulty during the operation of plating by electrical methods, in some cases due to the impurity itself plating and so causing the deposit to be impure and of less value, and in other cases due to the impurity bringing about a lowered efficiency in the plating process, is a fact well known in the arts. Consequently, great pains are taken and much expense is incurred in purifying electrolytes so that the harmful impurities may be removed to a sufficient extent.

In the electrolytic process for the winning of zinc, for example, the impurities cadmium, copper, tin, arsenic, antimony, lead, and other elements, if left in the electrolyte, will deposit along with the zinc in the electrolytic cell and will render the zinc impure so that its value is decreased; other impurities, among which may be mentioned arsenic, antimony, tin, germanium, tellurium, selenium, iron, nickel, and cobalt, lower the efficiency of the electrolysis so that more current is used to produce a pound of metal than would be required if these elements were absent, and so their presence greatly increases the expense of the process. Commonly, two and sometimes three processes are used to remove these impurities. The iron, together with part of the copper, arsenic, antimony, tin, germanium, tellurium, selenium, and other metals, is precipitated by treating the electrolyte with zinc oxide, or roasted zinc ore, or lime, while air is blown through the solution. The resulting precipitate is removed by thickeners or filters. The solution is then treated with zinc dust, sometimes along with other reagents such as copper salts, and antimony, arsenic, tellurium, selenium, tin, cobalt, copper, cadmium, and other elements are precipitated and may be removed by filtration. Sometimes a third method is used to remove certain elements, as, for example, sometimes a nitroso-B-naphthol is used to remove cobalt.

Now, in the removal of impurities by means of zinc dust, it is well known in the art that the purifying action of zinc dust is increased if finely divided copper be present; commonly this finely divided copper is formed by precipitating it from the solution to be purified by the zinc dust. Further, the purifying action of the zinc is still further increased if antimony or arsenic be deposited

upon it: when zinc dust, together with copper and antimony, is used, the purifying action becomes great enough to precipitate certain metals, of which cobalt is an example, which are very difficult to precipitate otherwise.

We have discovered that tin may be used instead of antimony or arsenic, and that tin has certain advantages which make it to be preferred to either arsenic or antimony. In the first place, tin does not tend to dissolve in the purification process to as great an extent as does arsenic or antimony and if it does dissolve, it is more easily removed by further treatment. Secondly, tin does not bring about as great a lowering of current efficiency in the electro-deposition of zinc as does antimony; in this respect it is more similar to arsenic. Thus, if some of the metal does get into solution during the purification process, then tin is less dangerous than antimony. Thirdly, tin precipitates in such a form that the cake of zinc dust-copper-tin plus impurities is more easily filtered than the corresponding cakes produced when antimony or arsenic is used: this feature is extremely important if the purification is carried out by drawing the solution to be purified through a layer or cake of the purifying agent.

As an example of the use of our invention, we took a sample of zinc electrolyte which showed the following analysis as to impurities:

|          | Milligrams per liter |
|----------|----------------------|
| Cobalt   | 7.9                  |
| Arsenic  | 0.12                 |
| Antimony | 0.03                 |
| Tin      | Trace                |

We dissolved 0.277 gram of stannous chloride and 8 grams of copper sulphate in water and then added 200 grams of zinc dust which passed a 20-mesh screen and was caught in a 48-mesh screen. The mixture was agitated until the copper was precipitated, then the supernatant liquid was decanted off. The zinc dust, coated with copper and tin, was then packed into a 1-inch copper tube about 12 inches long and held in place with glass wool. Arrangements were made so that the electrolyte could be drawn through this copper tube. The electrolyte was heated to 50° C. and drawn through; the contact time of the electrolyte with the mixture is estimated to have been 0.44 minutes. The issuing solution had the following analysis:

|                    | Milligrams per liter |
|--------------------|----------------------|
| Cobalt             | 1.5                  |
| Arsenic, less than | 0.01                 |
| Antimony           | 0.02                 |
| Tin                | Trace                |

That the tin plays an essential role in the purification was proved by carrying out the same experiment, using zinc dust alone, or zinc dust and copper only, and the same electrolyte. With zinc alone, the issuing solution had the analysis:

|          | Milligrams per liter |
|----------|----------------------|
| Cobalt   | 7.9                  |
| Arsenic  | 0.06                 |
| Antimony | 0.03                 |

With zinc dust coated with copper, the issuing solution had the analysis:

|                    | Milligrams per liter |
|--------------------|----------------------|
| Cobalt             | 6.1                  |
| Arsenic, less than | 0.01                 |
| Antimony           | 0.01                 |

It will be observed that in the precipitants above described, including zinc coated with copper, the precipitant in a finely divided form is

held in a porous bed, which has the effect of holding the precipitated impurities in contact with the purifying agent, by which means a degree of improved purification is obtained.

5 What we claim is:

1. In the purification of zinc electrolytes by means of metallic precipitants: the step of contacting the electrolyte with zinc dust coated with copper and tin as the precipitant.

10 2. A method of purifying zinc electrolytes by means of metallic precipitants comprising passing the electrolyte through a stationary porous mass of finely divided precipitant for the electrolyte comprising zinc dust coated with copper and tin, and maintaining the precipitated impurities in contact with the precipitants while continuing to pass the electrolyte through said mass.

DINSMORE LAURENCE GRIFFITH.  
LUTHER GLENN HENDRICKSON.